

April 30, 1935.

O. C. ROHDE

1,999,784

UNITING PARTS

Filed Feb. 28, 1933

2 Sheets-Sheet 1

*Fig. 1*



*Fig. 2*



*Fig. 3*



*Fig. 4*



*Fig. 5*



*Fig. 6*



Inventor

Otto C. Rohde

By Owner & Owner

Attorneys

April 30, 1935.

O. C. ROHDE

1,999,784

UNITING PARTS

Filed Feb. 28, 1933

2 Sheets-Sheet 2

Fig. 7



Fig. 8



Fig. 10



Fig. 9



Fig. 12



Fig. 11



Inventor

Otto C. Rohde

By *Omer & Omer*

Attorneys

## UNITED STATES PATENT OFFICE

1,999,784

## UNITING PARTS

Otto C. Rohde, Toledo, Ohio, assignor to Champion Spark Plug Company, Toledo, Ohio, a corporation of Delaware

Application February 28, 1933, Serial No. 658,975

9 Claims. (Cl. 219—10)

This invention relates to uniting parts, and more particularly to securing parts together by forming in situ therebetween a casting of manganese steel. Minor objects and details of the 5 invention will appear as the description proceeds.

In the accompanying drawings forming a part of this specification, Figure 1 is a view partly in section illustrating the first step in securing a spark plug core within its shell;

10 Figure 2 is similar to Figure 1, but showing the completed operation;

Figure 3 is an elevation of the sleeve shown in section in Figure 1 for uniting the core and shell;

15 Figure 4 is a cross section illustrating the securing of a disc in a socket in the end of a tube;

Figure 5 is a section similar to Figure 4 but showing the completion of the operation;

20 Figure 6 is an elevation of the securing sleeve shown in section in Figure 4;

Figure 7 is a section showing the securing of a collar upon a rod;

25 Figure 8 is a section similar to Figure 7 but showing the completion of the step;

Figure 9 is a view showing the initial step in securing a conducting rod within a socket in a non-conducting member;

30 Figure 10 is a view showing the completion of the operation illustrated in Figure 9;

Figure 11 is a view showing the first step in securing a hub or the like upon a shaft;

35 Figure 12 is a view showing the completion of the operation initiated in Figure 11.

In the construction shown in Figure 1, a spark 40 plug core 20 is seated within a shell 21 having in its upper end a counterbore 22. Between the shell and the core and in counterbore 22 there is inserted the inner end of a securing member 23. The inner end of the securing member is 45 tapered or reduced in cross section at 24 where it rests upon the shoulder 25 at the inner end of counterbore 22. The outer end 26 of member 23 is increased in thickness and is arranged to fit fairly closely within the upper end 27 of counterbore 22.

Midway in its length the counterbore 22 is somewhat enlarged, as by groove 28. Opposite the counterbore the surface of core 20 is tapered slightly as shown at 29.

50 With the parts assembled as shown in Figure 1, electric contact is made with the outer end of the member 23, as indicated by arrow 30. Also electric contact is made with the shell as indicated at 31. Thereupon electric current is passed between these contacts through the reduced por-

tion 24 of the sleeve. Since the cross section through which the current is passed is smallest at this point, the electric resistance is highest in the tapered portion 24. Member 23 is preferably of iron base metal, which may be manganese steel, and has sufficient resistance so that the temperature may be raised to the melting point by the electric current passed therethrough.

5 The electric current is continued and pressure is exerted upon the upper end 26 so that, as the inner end of the member melts, the outer end is crowded down until it rests within the upper end 27 of the counterbore, as shown in Figure 2. The molten metal of course flows outward into groove 28, forming a locking ring 32, as shown in Figure 2, and at the same time is pressed into intimate contact with the tapered side 29, as shown at 33 in Figure 2.

10 It is desirable to have the melting of the member 23 proceed progressively from its lower end upward during the melting operation. The member might be made tapered throughout, but in the example shown it is provided with successive shoulders, there being one shoulder at the bottom end of portion 26, and another shoulder 15 34 between that point and the bottom portion 24.

15 In Figures 4 and 5 there is shown the securing of a disc 35 within a socket 36 in the end of a tube 37. The socket 36 is larger than disc 35, to provide space for a fastening member. The fastening member comprises a body portion 38 having a shoulder 39 adapted to contact the outer side of disc 35 when the securing operation is completed. A reduced portion 40 of the member extends downward between the disc and the walls of socket 36, portion 40 being beveled at 41 where it rests upon the inner end of the socket. The outer end of the securing member is enlarged at 42 so as to make a close fit within the outer end 43 of socket 36. The inwardly extending portion 40 is shown provided with two steps or shoulders 44 and 45 which successively decrease the thickness of the wall towards the inner end. As will be seen from Figure 5, the inwardly extending portion 40 is melted and pressed downward so that it fills socket 36 at 46, as shown in Figure 5, and also is pressed outward at 47 into a groove 48 in the wall of the socket. This is accomplished by making electric contact with portion 42, as indicated by arrow 49, and contact with member 37, as indicated by arrow 50. When the current is passed between these contacts and pressure is exerted upon portion 42, portion 40 is progressively melted and pressed into contact 20 25 30 35 40 45 50 55 with the outer surface of disc 35 and the walls of

5

10

15

20

25

30

35

40

45

50

55

- socket 36. The parts are so proportioned that when shoulder 39 is pressed firmly against the outer edge of disc 35, the molten metal will be under pressure against the outer wall of the disc 5 and the wall of the socket. If there should be a slight excess of metal in portion 40, it will be readily understood that it would be extruded between shoulder 39 and the disc until firm contact is made by the shoulder with the disc. 10 Upon the solidification of the metal, it will be readily understood that the parts are firmly united.

In Figure 7 there is shown the uniting of a rod 51 with a sleeve 52. In this instance the sleeve 52 is provided with a socket 53 having a groove 54 therein. Within this socket 53 there is positioned a uniting member 55 having an enlarged outer end 56 which just fits within the outer end 57 of the socket. The inner end of member 55 is beveled at 58 and rests upon the inner end of the socket. With the parts assembled as shown at 57, electric contact is made with part 56, as indicated by arrow 59, and with sleeve 52, as indicated by arrow 60. When an electric current is passed between these contacts, it melts portion 55 progressively upward from the beveled end 58 to its upper end, and the melted metal is pressed outward into groove 54, as shown at 61 in Figure 8. Member 51 is also shown with a depression 62 therein into which the molten metal is pressed, as indicated at 63 in Figure 8. Member 51 may be of vitreous or similar material which might be subject to cracking if subjected to violent temperature changes at a sharp shoulder, such as is presented by groove 54. Therefore, depression 63 is rounded or curved inward so as to avoid any sharp edge. In this connection, it may be pointed out that also in Figure 1 the insulating core 20 is shaped so that it does not present any sharp corners to the molten metal.

In Figure 9 there is illustrated the securing of a conducting member 64 within a non-conducting member 65. The end of member 64 may be provided with a groove 66 and is shown resting upon a conducting disc 67 in the inner end of a socket 68 in member 65. A securing sleeve 69 is inserted between members 64 and 65 and has a thickened outer end 70 which will fit within outer end 71 of socket 68. The socket 68 is shown with a curving enlargement 72. Member 79 is beveled or reduced in cross section at 73 where it rests upon disc 67.

With the parts assembled as shown in Figure 9, electric contact is made with member 64, as indicated by arrow 74, and with portion 70 of member 69, as indicated by arrow 75. Current is passed between these contacts through members 64, 67 and 69. The point of greatest resistance is beveled portion 73 of member 69, and the current employed is sufficient to melt member 69 at this point and to continue to melt it progressively, as portion 70 is pressed downward, until the socket is completely filled, as indicated in Figure 10, whereupon the molten metal is pressed into groove 66, as shown at 76, and into enlarged portion 72 of the socket, as shown at 77. The molten material, solidifying in this position, permanently unites the parts.

In Figures 11 and 12 there is shown a method of securing a hub or the like 80 upon a shaft 81. The opening 82 within the hub is made somewhat larger than the shaft so that a sleeve 83 may be inserted between the shaft and hub. The central portion 84 of this sleeve is made the thinnest, with

increasing thickness on each side, as indicated at 85, and with the outer ends 86 of a size to closely fit within the hub. Electrical contact is made with each end of the sleeve, as indicated by arrows 87, and electric current is passed through the sleeve and melts the thinner intermediate portion and progressively outward while the thickened ends 86 remain solid and are pressed together and slip within the space between the hub and shaft. In this case there are no specific grooves shown in the respective members, although they may be employed, if desired. Very small depressions are sufficient to accomplish the desired purpose, the grooves illustrated in the other views being unnecessarily large, for purposes of illustration. As a matter of fact, a hub 10 united to a sleeve, as shown in Figures 11 and 12, will ordinarily remain firmly united against all ordinary forces to which they will be subjected, as 15 very minute irregularities in the respective surfaces are sufficient to hold them in exact position with respect to the uniting metal.

It will be seen that in each case the molten metal is forced into contact with the parts to be united and can be readily held under pressure 25 while it is being solidified. An iron base metal, which may be manganese steel, is preferred, because it may be readily given sufficient resistance to result in melting by an electric current, and furthermore it combines the quality of slightly 30 expanding upon solidification with very satisfactory strength after solidification.

It will be readily understood that in one of its broadest aspects my invention might be susceptible of use with widely different materials for uniting purposes, provided the proper conditions of electrical resistance are secured. Another broad aspect is the melting of the inner portion of the uniting element while the outer portion remains solid and is used as a plunger to press the molten 40 portion into position and maintain it under pressure while setting. For this purpose the outer portion of the united part is preferably made a good fit within the socket or space into which it is inserted. Any slight play around the outer 45 solid plunger portion of the uniting part will be quickly sealed by the chilling of molten material which starts to flow therethrough.

As a usual thing it is preferable to provide at least the outer portion of the socket with some 50 slight non-conducting film, such as a black finish, in order to minimize danger of short circuiting from the outer end of the uniting member through the surrounding member instead of forcing the electricity to pass through the uniting member. This of course applies only where the surrounding member is of conducting material. Where the conductor is within the uniting part, as shown in Figure 9 for example, it may be preferable to coat the outside of such conducting 55 member with a similar non-conducting film.

While I have shown several ways in which the invention may be applied to the uniting of different parts, it will be recognized that many other 60 modifications can be made within the scope of the invention as defined by the appended claims.

What I claim is:—

1. The method of uniting parts, which consists in assembling the parts to provide a sealing 70 space therebetween, introducing a solid filler into said space, said filler having less electric resistance at an outer end than at a point within the space, passing an electric current through said filler and thereby melting it within the space 75

while maintaining said outer end solid, pressing said outer end toward said space, as the filler melts, and into the outer end of said space to exert pressure on the molten filler, and continuing said pressure until the molten filler solidifies.

5. A method in accordance with claim 1 and in which the filler is of iron-base metal.

6. A method in accordance with claim 1 and in which the filler is of manganese steel.

10. 4. The method of uniting parts, at least one of which is of conducting material, said method consisting in assembling the parts with a sealing pocket therebetween, inserting into said pocket an iron-base member longer and thinner than said pocket, and making electric contact between the inner end of said member and one of said parts of conducting material, passing an electric current through said member and contacting part and melting the member from its inner end outwardly towards its outer end, pressing the unmelted outer end of the member into the pocket during said melting and thereby filling the pocket, and solidifying the molten metal in said pocket.

15. 5. A method in accordance with claim 4 and in which said filling member is of manganese steel.

20. 6. The method of securing a surrounding part upon a rod, which consists in assembling the rod

and part with an annular space therebetween, inserting a sleeve into said space, said sleeve having greater electrical resistance at an intermediate point than at its ends, making electric contact with the two ends of the sleeve and pressing them towards each other while passing through the sleeve an electric current sufficient to melt the intermediate portion of the sleeve, thereby filling the intermediate portion of the annular space with molten material, and solidifying said molten material while under pressure, to secure said part upon said rod.

25. 7. A method in accordance with claim 6 and in which said sleeve is of manganese steel.

8. The method of securing a disc in a socket larger in diameter than said disc, which comprises inserting into the socket around the disc the end of a sleeve which has an internal flange at its outer end adapted to overlie the edge of said disc, passing an electric current through said sleeve while pressing on its outer end until the inner end of the sleeve is melted and said flange presses firmly upon said disc, and then solidifying the molten material to hold the disc in place.

9. A method in accordance with claim 8 and in which the sleeve is of manganese steel.

OTTO C. ROHDE.